# EUROPEAN PATENT SPECIFICATION

(11) **EP 3 205 741 B1**
(45) Date of publication and mention of the grant of the patent: **05.04.2023**
(21) Application number: 15848228.1
(22) Date of filing: 16.09.2015
(51) Int. Cl.: C23C 2/20, C22C 18/04, C23C 2/06

(54) **CONTINUOUS HOT-DIP METAL PLATING METHOD AND CONTINUOUS HOT-DIP METAL PLATING EQUIPMENT**
KONTINUIERLICHES SCHMELZTAUCHVERFAHREN UND AUSRÜSTUNG FÜR KONTINUIERLICHES SCHMELZTAUCHVERFAHREN
PROCÉDÉ DE MÉTALLISATION PAR IMMERSION À CHAUD EN CONTINU ET MATÉRIEL DE MÉTALLISATION PAR IMMERSION À CHAUD EN CONTINU

(30) Priority: 08.10.2014 JP 2014206882
(43) Date of publication of application: 16.08.2017
(73) Proprietor: JFE Steel Corporation, Tokyo 100-0011 (JP)
(72) Inventor: TERASAKI, Yu, Tokyo 100-0011 (JP); TAKAHASHI, Hideyuki, Tokyo 100-0011 (JP); MIYAKE, Masaru, Tokyo 100-0011 (JP); YASUFUKU, Yusuke, Tokyo 100-0011 (JP); KOYAMA, Takumi, Tokyo 100-0011 (JP); INABA, Atsushi, Tokyo 100-0011 (JP); SASAKI, Masato, Tokyo 100-0011 (JP)
(74) Representative: Haseltine Lake Kempner LLP
(86) International application number: PCT/JP2015/004715
(87) International publication number: WO 2016/056178

(56) References cited:
- EP-A1- 0 707 897
- EP-A1- 1 466 994
- WO-A1-2014/135753
- JP-A- H09 195 024
- JP-A- H09 195 024
- JP-A- S54 135 628
- JP-A- 2007 302 959
- JP-A- 2014 055 307

## Description

### Technical Field

The present invention relates to a continuous hot-dip metal coating method, and a continuous hot-dip metal coating facility.

### Background Art

In a continuous hot-dip coating process, as shown in Fig. 4, a steel strip 1 from inside a snout 2 enters a molten metal 4 in a coating tank 3, has its direction changed by a sink roll 5, and is withdrawn from the coating tank 3. Then a gas wiping nozzle 6 disposed above the coating tank 3 wipes away excessive molten metal so that the coating weight is controlled to a predetermined level and the molten metal adhering on the surfaces of the steel strip 1 is leveled out in the strip transversal direction and strip longitudinal direction. The gas wiping nozzle 6 is usually configured to be longer than the steel strip width in order to accommodate various steel strip widths and to manage misalignment in the transversal direction during withdrawal of the steel strip, and so on, and extends outward beyond the transversal end portions of the steel strip 1.

In such a gas wiping method, the steel strip undergoes minute vibrations and the coating layer flows in an irregular manner due to blowing of the wiping gas, which frequently causes formation of a wavy pattern called bath wrinkles (also known as bath sagging) in the coating surface. If a coated steel sheet with bath wrinkles is used in outer panels such that the coating surface is used as a paint base surface, the surface properties of the paint film, smoothness in particular, are adversely affected. Thus, coated steel sheets with bath wrinkles cannot be used in outer panels that should be suitable for a painting process that gives excellent appearance, and the yield of the coated steel sheets is significantly affected.

To address the above-described issues, the following methods have been proposed to prevent bath wrinkle defects, which are appearance defects, of hot-dip metal-coated steel sheets.

A method described in Patent Literature 1 involves changing the surface properties of a temper rolling roll and rolling conditions during performance of temper rolling, which is the step subsequent to the steel sheet coating step, so that bath wrinkles are less conspicuous. A method described in Patent Literature 2 involves adjusting the surface roughness of a steel sheet according to the coating weight by using a skin-pass mill and a tension leveler, etc., prior to introducing the steel sheet into the molten zinc bath so as to reduce occurrence of bath wrinkles. Patent Literature 3 describes a method that involves setting the line speed and the height of the wiping nozzle from the bath surface that are optimum for the sheet thickness so as to reduce occurrence of bath wrinkles.

### Citation List

### Patent Literature

PTL 1: Japanese Unexamined Patent Application Publication No. 2004-27263
PTL 2: Japanese Unexamined Patent Application Publication No. 55-21564
PTL 3: Japanese Unexamined Patent Application Publication No. 9-41113

Documents WO2014/135753A1 and JP-H 09195024A disclose continuous hot-dip coating methods wherein conditions of the gas wiping step are controlled. Documents JP2014 055307-A, and EP0707897 A1 disclose methods and systems for controlling the coating thickness in methods for continuous hot-dip coating by adjusting the wiping gas.

### Summary of Invention

### Technical Problem

However, according to the studies made by the inventors of the present invention, although minor bath wrinkles are overcome by the method described in Patent Literature 1, the method has had no effect on severe bath wrinkle defects. According to the method described in Patent Literature 2, a skin-pass mill, a tension leveler, and other facilities are needed to be installed for the process before the molten zinc bath, which poses a problem of cost. Even when these facilities are installed, ideal surface roughness is rarely obtained due to chemical and/or physical changes caused by pickling and recrystallization in pre-treatment facilities and annealing furnaces, which presumably makes it difficult to completely prevent occurrence of bath wrinkles. Moreover, according to the method described in Patent Literature 3, the line speed and the wiping nozzle height cannot immediately follow the changing point of the sheet thickness and thus steel sheets with bath wrinkles are inevitably produced, which leads to yield loss.

The present invention has been made under the circumstances described above and aims to provide a continuous hot-dip metal coating method that uses a gas wiping nozzle to control the coating weight and prevents occurrence of bath wrinkle defects so that high-quality hot-dip metal-coated steel strips can be stably manufactured at a low cost. The present invention also aims to provide a galvanized steel strip and a continuous hot-dip metal coating facility.

### Solution to Problem

The invention is defined in the independent claims.

### Advantageous Effects of Invention

According to the present invention, occurrence of coating surface defects called bath wrinkles is suppressed and high-quality hot-dip metal-coated steel strips can be stably produced at a low cost.

### Brief Description of Drawings

[Fig. 1] Fig. 1 is a schematic view of a production facility for a continuous hot-dip metal-coated steel strip according to an embodiment of the present invention.
[Fig. 2] Fig. 2 is an enlarged view of a tip of a gas wiping nozzle according to an embodiment of the present invention.
[Fig. 3] Fig. 3 is a graph showing whether bath wrinkles occurred in relation to the relationship between a D/B value and a wiping gas temperature T.
[Fig. 4] Fig. 4 is a schematic diagram of a conventional production facility for a continuous hot-dip metal-coated steel strip.

### Description of Embodiments

The present invention will now be specifically described.

A continuous hot-dip metal coating facility according to the present invention is a facility used in continuously dipping a steel strip in a coating bath of a hot-dip metal coating tank so as to conduct a coating treatment, and then withdrawing the steel strip from the coating bath and blowing wiping gas toward the coated steel strip from a gas wiping nozzle installed above the coating bath so as to adjust the coating metal weight. The continuous hot-dip metal coating facility according to the present invention includes a distance meter that measures a distance between a steel strip and a tip of a gas wiping nozzle in a non-contact manner, a control unit that calculates a target temperature T of wiping gas to be injected from the gas wiping nozzle on a basis of a distance D measured by the distance meter and a gap B of the gas wiping nozzle, and a gas heating device that heats the gas to be injected from the gas wiping nozzle to the target temperature T calculated by the control unit.

Fig. 1 illustrates a continuous hot-dip metal coating apparatus according to an embodiment of the present invention. In Fig. 1, 1 denotes a steel strip, 2 denotes a snout, 3 denotes a coating tank, 4 denotes a molten metal, 5 denotes a sink roll, 6 denotes a gas wiping nozzle, 7 denotes a distance meter, 8 denotes a control unit (CU), and 9 denotes a gas heating device. The arrow indicates the direction in which the steel strip 1 is moved. The steel strip 1 from inside the snout 2 enters the molten metal 4 in the coating tank 3, has its direction changed by the sink roll 5, and is withdrawn from the coating tank 3. Then excess molten metal is wiped away by the gas wiping nozzle 6 installed above the coating tank 3 so that the coating weight is controlled to a predetermined weight.

Fig. 2 is an enlarged view of a tip of the gas wiping nozzle 6. In the present invention, the distance between the tip of the gas wiping nozzle 6 and the steel strip 1 is indicated by D for the sake of convenience. The gas wiping nozzle 6 includes an upper nozzle part 6a and a lower nozzle part 6b and the gap in the gas wiping nozzle 6 is indicated by B.

The distance meter 7 is, for example, installed below the gas wiping nozzle 6. The distance meter 7 continuously measures the distance D between the tip of the gas wiping nozzle 6 and the steel strip 1 and inputs the reading to the control unit 8. The control unit 8 calculates a target temperature of the wiping gas to be heated with the gas heating device 9 on a basis of the measurement data of the distance D input from the distance meter 7. The gas heating device 9 heats the wiping gas to the target temperature calculated by the control unit 8 and supplies the heated wiping gas to the gas wiping nozzle 6. The distance meter 7 may be any non-contact meter. The type of the control unit 8 is not particularly limited. The type of the gas heating device 9 is also not particularly limited as long as the device has a function of heating the wiping gas without delay based on the distance D between the gas wiping nozzle 6 and the steel strip 1. The gas heating device 9 may employ any method for heating the wiping gas to be supplied to the gas wiping nozzle 6. Examples of the method include a method of supplying gas heated by a heat exchanger and a method of mixing flue gas from the annealing furnace and air.

In the present invention, the temperature T of the wiping gas injected from the gas wiping nozzle 6 is controlled on a basis of a D/B value, which is the ratio of the distance D between the tip of the gas wiping nozzle 6 and the steel strip 1 to the gap B of the gas wiping nozzle 6. Since the temperature T of the wiping gas is controlled on the basis of the D/B value, flowability of the molten metal is improved. As a result, the molten metal flows down regularly and an effect of preventing bath wrinkle defects can be fully exhibited.

In the present invention, the wiping gas injected from the gas wiping nozzle 6 is an inert gas. With inert gas, oxidation of the molten metal on the steel sheet surface can be prevented and the flowability of the molten metal can be further improved. Examples of the inert gas include, but are not limited to, nitrogen, argon, helium, and carbon dioxide.

When the temperature of the wiping gas is excessively low, bath wrinkle defects caused by low flowability of the molten metal occur. When the temperature of the wiping gas is excessively high, alloying is promoted and the appearance of the steel sheet is deteriorated. Thus, there is need to select the temperature T of the wiping gas optimum for the D/B value. In this respect, in the present invention, the relationship between the D/B value and the temperature T of the wiping gas for obtaining products free of bath wrinkle defects and having good appearance is determined. Assuming that the temperature of the molten zinc bath is 460°C, the line speed is 100 m/min, the pressure of the nozzle header is 30 kPa, and the gas type is air, a steel strip having a thickness of 1.2 mm and a width of 1000 mm is threaded through the continuous hot-dip metal coating facility. As a result, the relationship shown in Fig. 3 is obtained. In Fig. 3, the evaluation standards related to the state of occurrence of the bath wrinkles were as follows where Wa denotes the arithmetic mean waviness Wa [µm] measured in accordance with the JIS B0601-2001 standard.
F: Fail, galvanized steel sheet with large visually recognizable bath wrinkles (1.50 < Wa)
C: Fail, galvanized steel sheet with small visually recognizable bath wrinkles (1.00 < Wa ≤ 1.50)
A: Pass, aesthetically pleasing galvanized steel sheet free of visually recognizable bath wrinkles (0.50 < Wa ≤ 1.00)

The results in Fig. 3 show that the temperature T of the wiping gas is controlled to be in the range indicated by formula (1) below according to the D/B value.
[Math. 1] ${c}_{1} \sqrt{\frac{D}{B}} - {c}_{2} \frac{D}{B} + {T}_{M} - 100 ≦ T ≦ {c}_{1} \sqrt{\frac{D}{B}} + {c}_{3} \frac{D}{B} + {T}_{M} + 100$
T: the temperature of the wiping gas injected from the gas wiping nozzle [°C]
T_{M}: melting point of molten metal [°C]
D: distance between the steel strip and the tip of the gas wiping nozzle [m]
B: gas wiping nozzle gap [m]
c₁, c₂, and c₃: constants

Since the constants c₁, c₂, and c₃ in the formula (1) change depending on the size of the wiping nozzle gap B and the nozzle shape, they must be determined preliminarily offline. Specifically, a thermometer is set to a sheet surface simulating a steel strip and the reading of the thermometer is assumed to be the "temperature of the wiping gas at an impinging position where the wiping gas impinges on the steel strip". Some conditions for the D/B value are changed and the temperature is measured to determine the values of c1 to c3.

Since the wiping gas has substantially no wiping power at a D/B exceeding 60, there is no need to heat the wiping gas. In this respect, the upper limit of the D/B value is 60 or less.

In the present invention, the temperature of the wiping gas at an impinging position where the wiping gas impinges on the steel strip is set to be within a 200°C range below and above the melting point T_{M}(T_{M} ∓100 °C) of the molten metal. When the temperature of the wiping gas at the impinging position where the wiping gas impinges on the steel strip is lower than (T_{M} - 100)°C, the ratio of metal solidified from the molten metal adhering on the steel sheet is significantly increased, the flowability of the molten metal is thus degraded, and bath wrinkle defects occur. For example, when a heat exchanger is used, the temperature of gas or liquid at the heating side may be changed to control the temperature of the wiping gas at the heated side. However, the method of control is not limited to this.

Meanwhile, when the temperature of the wiping gas at the impinging position where the wiping gas impinges on the steel strip exceeds (T_{M} + 100)°C, alloying of the steel strip and the molten metal is accelerated, appearance of the steel sheet is degraded, and the coating weight becomes higher than what is targeted. Moreover, since extra energy is consumed to heat the gas, energy efficiency is also degraded. As shown by Fig. 5 in Non-Patent Literature 1 (The Journal of the Iron and Steel Institute of Japan, vol. 81 (1995), No. 2, p. 49), it is known that the potential core of the wiping gas attenuates in proportion to the D/B value; hence, an appropriate gas temperature must be set according to the D/B value.

Since the melting point changes with changes in the composition of the molten metal coating (coating layer), the optimum range for the wiping gas temperature T varies.

In the case of a galvanized steel strip having an Al-Zn based coating layer at the steel strip surface, the Al-Zn coating layer containing Al: 1.0% to 10% by mass, Mg: 0.2% to 1.0% by mass, Ni: 0.005% to 0.10% by mass, and the balance being Zn and unavoidable impurities, Mg, which is more readily oxidizable than Al and Zn, is contained. Thus, it has been confirmed that when the wiping gas temperature is low, the flowability of the molten metal is particularly degraded and bath wrinkles easily occur. As a result, the surface appearance is degraded. In this respect, optimizing the wiping gas temperature to achieve a bath wrinkle defect preventing effect is particularly preferable for a galvanized steel strip produced by the gas wiping method of the present invention and having an Al-Zn based coating layer at the steel strip surface, the Al-Zn coating layer containing Al: 1.0% to 10% by mass, Mg: 0.2% to 1.0% by mass, Ni: 0.005% to 0.10% by mass, and the balance being Zn and unavoidable impurities.

### EXAMPLE 1

A galvanized steel strip production test was conducted to study optimum installation conditions and embodiments of the gas wiping nozzle. A gas wiping nozzle having a nozzle gap B of 1.2 mm was used. The gas wiping nozzle height from the molten zinc bath surface was set at 350 mm and the wiping gas injection direction was set to be perpendicular to the steel strip surface. Specifically, a steel strip having a thickness of 1.2 mm and a width of 1000 mm was threaded at a line speed of 100 m/min and the composition of the coating layer, the distance D between the tip of the gas wiping nozzle and the steel strip, the pressure of gas injected from the gas wiping nozzle (nozzle header pressure), the gas set temperature, the gas type, and the coating weight were varied for evaluating the appearance of the steel sheet. The molten zinc bath temperature was set at 460°C. The constants in formula (1) were determined in advance through off-line testing and were c₁ = 45, c₂ = 1.5, and c₃ = 2.5.

The method for supplying gas to the gas wiping nozzle was a method that included heating room-temperature gas to a predetermined temperature with a heat exchanger and compressing the gas to a predetermined pressure by using a blower. The melting point (T_{M}) of the molten metal was T_{M} = 420°C when Al = 0.2% by mass and was T_{M} = 375°C when Al = 4.5% by mass, Mg = 0.5% by mass, and Ni = 0.05% by mass.

The appearance of the steel sheet was evaluated according to the following standards. Wa is the value of the arithmetic mean waviness Wa [µm] measured in accordance with the JIS B0601-2001 standard.
F: Fail, galvanized steel sheet with large visually recognizable bath wrinkles (1.50 < Wa)
C: Fail, galvanized steel sheet with small visually recognizable bath wrinkles (1.00 < Wa ≤ 1.50)
A: Pass, aesthetically pleasing galvanized steel sheet free of visually recognizable bath wrinkles (0.50 < Wa ≤ 1.00)
AA: Pass, highly aesthetically pleasing galvanized steel sheet free of visually recognizable bath wrinkles (0 < Wa ≤ 0.50)

The results are shown in Table 1. Note that Examples 1-9 are not in conformity with the steel strip of claim 2. Examples 1-8 are also not in conformity with the method of claim 1.

**[Table 1]**

| | Nozzle header pressure [kPa] | Gas set temperature [°C] | Gas type | Coating layer composition [mass%] | | | | Nozzle-steel strip distance D [mm] | Nozzle gap B [mm] | D/B [-] | Optimum gas temperature range derived from D/B value [°C] | Coating weight [g/m²] | Appearance | Wa [µm] |
|---|---|---|---|---|---|---|---|---|---|---|---|---|---|---|
| | | | | Al | Mg | Ni | Zn | | | | | | | |
| Example 1 | 30 | 550 | Air | 0.2 | 0 | 0 | Balance | 25 | 1.2 | 20.83 | 494-777 | 130 | A | 0.73 |
| Example 2 | 30 | 600 | Air | 0.2 | 0 | 0 | Balance | 30 | 1.2 | 25.00 | 508-808 | 125 | A | 0.64 |
| Example 3 | 30 | 590 | Air | 0.2 | 0 | 0 | Balance | 4 | 1.2 | 3.33 | 397-610 | 56 | A | 0.86 |
| Example 4 | 30 | 420 | Air | 0.2 | 0 | 0 | Balance | 6 | 1.2 | 5.00 | 413-633 | 64 | A | 0.74 |
| Example 5 | 30 | 670 | Air | 0.2 | 0 | 0 | Balance | 17 | 1.2 | 14.17 | 468-725 | 102 | A | 0.88 |
| Example 6 | 30 | 740 | Air | 0.2 | 0 | 0 | Balance | 45 | 1.2 | 37.50 | 539-889 | 142 | A | 0.53 |
| Example 7 | 30 | 610 | Air | 0.2 | 0 | 0 | Balance | 56 | 1.2 | 46.67 | 557-944 | 156 | A | 0.79 |
| Example 8 | 30 | 900 | Air | 0.2 | 0 | 0 | Balance | 58 | 1.2 | 48.33 | 560-954 | 167 | A | 0.68 |
| Example 9 | 30 | 550 | Nitrogen | 0.2 | 0 | 0 | Balance | 25 | 1.2 | 20.83 | 494-777 | 126 | AA | 0.08 |
| Example 10 | 30 | 550 | Nitrogen | 4.5 | 0.5 | 0.05 | Balance | 25 | 1.2 | 20.83 | 449-732 | 127 | AA | 0.12 |
| Comparative Example 1 | 30 | 420 | Air | 0.2 | 0 | 0 | Balance | 25 | 1.2 | 20.83 | 494-777 | 155 | C | 1.41 |
| Comparative Example 2 | 30 | 830 | Air | 0.2 | 0 | 0 | Balance | 25 | 1.2 | 20.83 | 494-777 | 163 | C | 1.25 |
| Comparative Example 3 | 30 | 770 | Air | 0.2 | 0 | 0 | Balance | 6 | 1.2 | 5.00 | 413-633 | 85 | C | 1.34 |
| Comparative Example 4 | 30 | 400 | Air | 0.2 | 0 | 0 | Balance | 15 | 1.2 | 12.50 | 460-710 | 114 | C | 1.30 |
| Comparative Example 5 | 30 | 820 | Air | 0.2 | 0 | 0 | Balance | 20 | 1.2 | 16.67 | 479-745 | 133 | C | 1.29 |
| Comparative Example 6 | 30 | 960 | Air | 0.2 | 0 | 0 | Balance | 48 | 1.2 | 40.00 | 545-905 | 171 | C | 1.21 |
| Comparative Example 7 | 30 | 490 | Air | 0.2 | 0 | 0 | Balance | 52 | 1.2 | 43.33 | 551-925 | 173 | C | 1.44 |
| Comparative Example 8 | 30 | 960 | Air | 0.2 | 0 | 0 | Balance | 7 | 1.2 | 5.83 | 420-643 | 108 | F | 1.67 |
| Comparative Example 9 | 30 | 860 | Air | 0.2 | 0 | 0 | Balance | 10 | 1.2 | 8.33 | 437-671 | 134 | F | 1.98 |
| Comparative Example 10 | 30 | 330 | Air | 0.2 | 0 | 0 | Balance | 21 | 1.2 | 17.50 | 482-752 | 136 | F | 1.72 |
| Comparative Example 11 | 30 | 360 | Air | 0.2 | 0 | 0 | Balance | 55 | 1.2 | 45.83 | 556-939 | 185 | F | 1.69 |
| Comparative Example 12 | 30 | 420 | Air | 4.5 | 0.5 | 0.05 | Balance | 25 | 1.2 | 20.83 | 449-732 | 149 | F | 1.88 |

In Example 1, bath wrinkle defects were prevented by performing wiping at an optimum gas temperature for the D/B value. The reasons bath wrinkle defects were prevented are presumably that wiping was performed at a gas temperature optimum for the D/B value and that the temperature of the wiping gas at the impinging position where the wiping gas impinged on the steel strip was set at (T_{M} - 100)°C or higher, which inhibited the cooling effect of the injected gas and caused the molten zinc on the steel sheet to remain relatively unsolidified and flow down regularly.

In Example 2, D/B was changed and wiping was performed at a wiping gas temperature T optimum for the changed value, thereby preventing bath wrinkle defects as in Example 1. In Examples 3 to 8, the results of changing the wiping temperature relative to the D/B values are shown.

In contrast, Comparative Example 1 and Comparative Example 2 are examples in which the gas temperature was outside the optimum gas temperature range derived from the D/B value. The reasons the coating weight increased in Comparative Example 1 were presumably that wiping was conducted at a temperature outside the optimum gas temperature range for the D/B value and that the temperature of the wiping gas at the steel strip impinging point was below (T_{M} - 100)°C due to mixing of ambient gas into the wiping gas injected from the nozzle. In Comparative Example 2, the temperature of the wiping gas was increased to be higher than in Example 1 and the coating weight increased. This is presumably because of an excessively high wiping gas temperature, which accelerates alloying of the zinc coating on the steel strip surface layer. Also, due to acceleration of alloying, the steel sheet surface became whitish in color and appearance was degraded. Results under other wiping conditions are indicated in Comparative Examples 3 to 11.

Example 10 and Comparative Example 12 are examples in which the composition of the coating layer was changed. Because the composition of the molten zinc was changed, the melting point of the zinc bath decreased to 375°C and thus the optimum temperature range of the wiping gas also changed. In Comparative Example 12, occurrence of larger bath wrinkles than in Comparative Example 1 was observed. This is probably because Mg in the coating layer composition is readily oxidable and bath wrinkles readily occurred as a result. In Example 10, the wiping gas temperature T was controlled and bath wrinkle defects were prevented as in Example 1.

In Examples 9 and 10, the type of gas was nitrogen, which is an inert gas, and thus better appearance was obtained than in Example 1.

As described above, a bath wrinkle defect preventing effect can be obtained by performing wiping at an appropriate wiping gas temperature.

### Reference Signs List

- 1: steel strip
- 2: snout
- 3: coating tank
- 4: molten metal
- 5: sink roll
- 6: gas wiping nozzle
- 6a: upper nozzle part of the gas wiping nozzle
- 6b: lower nozzle part of the gas wiping nozzle
- 7: distance meter
- 8: control unit (CU)
- 9: gas heating device

## Claims

1. A continuous hot-dip metal coating method comprising:
continuously immersing a steel strip (1) into a molten metal bath (3, 4) and
blowing gas from a gas wiping nozzle (6) onto the steel strip immediately after the steel strip is withdrawn from the molten metal bath so as to control a coating weight,
wherein a temperature T of wiping gas to be injected from the gas wiping nozzle (6) is controlled on a basis of a D/B value, which is a ratio of a distance D between a tip of the gas wiping nozzle and the steel strip to a gap B of the gas wiping nozzle,
wherein the temperature T of the wiping gas is controlled on a basis of the D/B value, wherein the D/B value is 60 or less, so as to be within a range of T_{M} ∓100°C °C at an impinging position where the wiping gas impinges on the steel strip, where T_{M} represents a melting point of molten metal in the molten metal bath (3, 4),
and wherein the temperature T of the wiping gas is controlled so as to be within a range indicated by formula (1) below:
[Math. 1] ${c}_{1} \sqrt{\frac{D}{B}} - {c}_{2} \frac{D}{B} + {T}_{M} - 100 ≦ T ≦ {c}_{1} \sqrt{\frac{D}{B}} + {c}_{3} \frac{D}{B} + {T}_{M} + 100$
T: the temperature of the wiping gas to be injected from the gas wiping nozzle [°C]
T_{M}: the melting point of the molten metal [°C]
D: the distance between the steel strip and the tip of the gas wiping nozzle [m]
B: the gap of the gas wiping nozzle [m]
c₁, c₂, and c₃: constants,
wherein the constants c1, c2 and c3 depend on the size of the wiping nozzle gap B and the nozzle shape, and wherein the constants c1, c2 and c3 are determined preliminarily offline by setting a thermometer to a sheet surface simulating a steel strip, changing conditions for the D/B value and measuring the temperature to determine the values of c1, c2 and c3, wherein the temperature measured by the thermometer is assumed to be the temperature of the wiping gas at an impinging position where the wiping gas impinges on the steel strip, wherein the wiping gas injected from the gas wiping nozzle is an inert gas.

2. A method for producing a galvanized steel strip, the steel strip comprising:
an Al-Zn based coating layer at a steel strip surface,
the Al-Zn based coating layer containing
Al: 1.0% to 10% by mass,
Mg: 0.2% to 1.0% by mass,
Ni: 0.005% to 0.10% by mass, and
the balance being Zn and unavoidable impurities; wherein a value of an arithmetic mean waviness Wa [µm] measured in accordance with the JIS B0601-2001 standard is 1.00 or lower; the method comprising the steps of the continuous hot-dip metal coating method according to Claim 1.

3. A continuous hot-dip metal coating facility arranged to perform the method of claim 1 or 2, the continuous hot-dip metal coating facility comprising:
a distance meter (7) that measures the distance D between the steel strip (1) and the tip of the gas wiping nozzle (6) in a non-contact manner,
a control unit (8) that calculates the target temperature T of wiping gas to be injected from the gas wiping nozzle (6), on the basis of the distance D measured by the distance meter (7) and the gap B of the gas wiping nozzle, such that the temperature T of the wiping gas is controlled on a basis of the D/B value, wherein the D/B value is 60 or less, so as to be within a range of T_{M} ∓100°C at an impinging position where the wiping gas impinges on the steel strip, where T_{M} represents a melting point of molten metal in the molten metal bath (3, 4), and
a gas heating device (9) that heats the gas to be injected from the gas wiping nozzle (6) in accordance with the target temperature T calculated by the control unit (8).

## Patentansprüche

1. Kontinuierliches Schmelztauch-Metallbeschichtungsverfahren, umfassend:
kontinuierliches Eintauchen eines Stahlbands (1) in ein Metallschmelzbad (3, 4) und
Blasen von Gas aus einer Gasabstreifdüse (6) auf das Stahlband unmittelbar nach Herausziehen des Stahlbands aus dem Metallschmelzbad, um ein Beschichtungsgewicht zu kontrollieren,
wobei eine Temperatur T des aus der Gasabstreifdüse (6) einzuspritzenden Abstreifgases auf Basis eines D/B-Werts gesteuert wird, der ein Verhältnis eines Abstands D zwischen einer Spitze der Gasabstreifdüse und dem Stahlband zu einem Spalt B der Gasabstreifdüse ist,
wobei die Temperatur T des Abstreifgases basierend auf dem D/B-Wert gesteuert wird, wobei der D/B-Wert 60 oder weniger ist, sodass er in einem Bereich von T_{M} ∓ 100 °C an einer Auftreffposition ist, an der das Abstreifgas auf das Stahlband auftrifft, wobei T_{M} einen Schmelzpunkt von geschmolzenem Metall in dem Metallschmelzbad (3, 4) darstellt,
und wobei die Temperatur T des Abstreifgases gesteuert wird, um innerhalb eines durch die nachstehende Formel (1) angegebenen Bereichs zu sein:
[Math. 1] ${c}_{1} \sqrt{\frac{D}{B}} - {c}_{2} \frac{D}{B} + {T}_{M} - 100 ≦ T ≦ {c}_{1} \sqrt{\frac{D}{B}} + {c}_{3} \frac{D}{B} + {T}_{M} + 100$
T: die Temperatur des Abstreifgases [°C], das aus der Gasabstreifdüse eingespritzt werden soll
T_{M}: der Schmelzpunkt des geschmolzenen Metalls [°C]
D: der Abstand zwischen dem Stahlband und der Spitze der Gasabstreifdüse [m] B: der Abstand der Gasabstreifdüse [m]
c₁, c₂, und c₃: Konstanten,
wobei die Konstanten c₁, c₂ und c₃ von der Größe des Abstreifdüsenspalts B und der Düsenform abhängen, und wobei die Konstanten c₁, c₂ und c₃ im Vorfeld offline bestimmt werden, indem ein Thermometer auf eine ein Stahlband simulierende Blechoberfläche gesetzt wird, die Bedingungen für den D/B-Wert geändert werden und die Temperatur gemessen wird, um die Werte von c₁, c₂ und c₃ zu bestimmen, wobei angenommen wird, dass die von dem Thermometer gemessene Temperatur die Temperatur des Abstreifgases an einer Auftreffposition ist, an der das Abstreifgas auf das Stahlband auftrifft, wobei das aus der Gasabstreifdüse eingespritzte Abstreifgas ein Inertgas ist. v

2. Verfahren zum Herstellen eines galvanisierten Stahlbands, das Stahlband umfassend:
eine Al-Zn basierte Beschichtungsschicht auf der Oberfläche eines Stahlbands,
wobei die Al-Zn basierte Beschichtungsschicht Folgendes enthält
Al: 1,0 % bis 10 % nach Masse,
Mg: 0,2 % bis 1,0 % nach Masse,
Ni: 0,005 % bis 0,10 % nach Masse, und
wobei der Rest Zn und unvermeidbare Verunreinigungen sind; wobei
ein Wert einer arithmetischen mittleren Welligkeit Wa [µm], gemessen gemäß der Norm JIS B0601-2001, 1,00 oder weniger ist; das Verfahren umfassend die Schritte des kontinuierlichen Schmelztauch-Metallbeschichtungsverfahrens gemäß Anspruch 1.

3. Kontinuierliche Schmelztauch-Metallbeschichtungsanlage, die angeordnet ist, um das Verfahren gemäß Anspruch 1 oder 2 auszuführen, die kontinuierliche Schmelztauch-Metallbeschichtungsanlage umfassend:
einen Abstandsmesser (7), der den Abstand D zwischen dem Stahlband (1) und der Spitze der Gasabstreifdüse (6) berührungslos misst,
eine Steuereinheit (8), die die Zieltemperatur T des aus der Gasabstreifdüse (6) einzuspritzenden Abstreifgases basierend auf dem von dem Abstandsmesser (7) gemessenen Abstand D und dem Spalt B der Gasabstreifdüse berechnet, sodass die Temperatur T des Abstreifgases basierend auf dem D/B-Wert gesteuert wird, wobei der D/B-Wert 60 oder weniger ist, sodass er an einer Auftreffposition, an der das Abstreifgas auf das Stahlband auftrifft, in einem Bereich von T_{M} ∓100 °C ist, wobei T_{M} einen Schmelzpunkt von geschmolzenem Metall in dem Metallschmelzbad (3, 4) darstellt, und
eine Gasheizvorrichtung (9), die das aus der Gasabstreifdüse (6) einzuspritzende Gas entsprechend der von der Steuereinheit (8) berechneten Solltemperatur T erwärmt.

## Revendications

1. Un procédé de revêtement métallique par immersion à chaud en continu comprenant :
l'immersion continue d'une bande d'acier (1) dans un bain de métal fondu (3, 4) et le soufflage de gaz à partir d'une buse d'essuyage de gaz (6) sur la bande d'acier immédiatement après que la bande d'acier ait été retirée du bain de métal fondu de manière à contrôler un poids de revêtement,
dans lequel une température T du gaz d'essuyage à injecter à partir de la buse d'essuyage de gaz (6) est contrôlée sur la base d'une valeur D/B, qui est un rapport d'une distance D entre une pointe de la buse d'essuyage de gaz et la bande d'acier à un écart B de la buse d'essuyage de gaz,
dans lequel la température T du gaz d'essuyage est contrôlée sur la base de la valeur D/B, dans lequel la valeur D/B est de 60 ou moins, de manière à être dans une plage de T_{M} ∓ 100 °C à une position d'impact où le gaz d'essuyage heurte la bande d'acier, où T_{M} représente un point de fusion du métal fondu dans le bain de métal fondu (3, 4),
et dans lequel la température T du gaz d'essuyage est contrôlée de manière à être dans une plage indiquée par la formule (1) ci-dessous :
[Math. 1] ${c}_{1} \sqrt{\frac{D}{B}} - {c}_{2} \frac{D}{B} + {T}_{M} - 100 ≦ T ≦ {c}_{1} \sqrt{\frac{D}{B}} + {c}_{3} \frac{D}{B} + {T}_{M} + 100$
T : la température du gaz d'essuyage à injecter à partir de la buse d'essuyage de gaz [°C]
T_{M} : le point de fusion du métal fondu [°C]
D : la distance entre la bande d'acier et la pointe de la buse d'essuyage du gaz [m] B : l'écart de la buse d'essuyage du gaz [m]
c1, c2 et c3 : constantes,
dans lesquelles les constantes c1, c2 et c3 dépendent de la taille de l'écart de la buse d'essuyage B et de la forme de la buse, et dans lesquelles les constantes c1, c2 et c3 sont déterminées hors ligne de manière préliminaire en plaçant un thermomètre sur une surface de feuille simulant une bande d'acier, en changeant les conditions pour la valeur D/B et en mesurant la température pour déterminer les valeurs de c1, c2 et c3, dans lequel la température mesurée par le thermomètre est supposée être la température du gaz d'essuyage à une position d'impact où le gaz d'essuyage heurte la bande d'acier, dans lequel le gaz d'essuyage injecté à partir de la buse d'essuyage de gaz est un gaz inerte.

2. Un procédé de production d'une bande d'acier galvanisée, la bande d'acier comprenant :
une couche de revêtement à base de Al-Zn sur une surface de la bande d'acier,
la couche de revêtement à base de Al-Zn contenant
Al : 1,0 % à 10 % en masse,
Mg : 0,2 % à 1,0 % en masse,
Ni : 0,005 % à 0,10 % en masse, et
le reste étant du Zn et des impuretés inévitables ; dans lequel une valeur d'une ondulation moyenne arithmétique Wa [µm] mesurée conformément à la norme JIS B0601-2001 est de 1,00 ou moins ; le procédé comprenant les étapes du procédé de revêtement métallique par immersion à chaud en continu selon la revendication 1.

3. Une installation de revêtement métallique par immersion à chaud en continu agencée pour réaliser le procédé selon la revendication 1 ou 2, l'installation de revêtement métallique par immersion à chaud en continu comprenant :
un télémètre (7) qui mesure la distance D entre la bande d'acier (1) et la pointe de la buse d'essuyage de gaz (6) d'une manière sans contact,
une unité de commande (8) qui calcule la température cible T du gaz d'essuyage à injecter à partir de la buse d'essuyage de gaz (6), sur la base de la distance D mesurée par le télémètre (7) et de l'écart B de la buse d'essuyage de gaz, de sorte que la température T du gaz d'essuyage est contrôlée sur la base de la valeur D/B, dans laquelle la valeur D/B est de 60 ou moins, de manière à être dans une plage de T_{M} ∓ 100 °C à une position d'impact où le gaz d'essuyage heurte la bande d'acier, où T_{M} représente un point de fusion du métal fondu dans le bain de métal fondu (3, 4), et
un dispositif de chauffage de gaz (9) qui chauffe le gaz à injecter depuis la buse d'essuyage de gaz (6) en fonction de la température cible T calculée par l'unité de commande (8).
